

# UNITED STATES PATENT OFFICE.

ANDREW THOMA, OF CAMBRIDGE, MASSACHUSETTS, ASSIGNOR TO NORTH AMERICAN CHEMICAL COMPANY, OF NEW YORK, N. Y., A CORPORATION OF MAINE.

## SHOE-FILLER.

1,227,696.

Specification of Letters Patent.

Patented May 29, 1917.

No Drawing. Original application filed May 11, 1908, Serial No. 432,083. Divided and this application filed July 1, 1912. Serial No. 707,018.

*To all whom it may concern:*

Be it known that I, ANDREW THOMA, a citizen of the United States, and resident of Cambridge, county of Middlesex, State of Massachusetts, have invented an Improvement in Shoe-Fillers, of which the following description is a specification.

My present invention relates to shoe fillers, and this application is a division of my former application Serial No. 432,083, filed May 11, 1908, now Patent No. 1,032,312, dated July 9, 1913. As disclosed in that application, which is in part a derivative of my foundation or pioneer filler Patent No. 832,002, September 25, 1906, I have found that several materials have qualities which adapt them for use as binders in shoe filling compositions, *i. e.* compositions used in filling the inner soles of shoes of certain kinds. These compositions are usually composed of cork or ground leather and a suitable binder. Wax tailings, a product of petroleum distillation, is such a binder, as stated in that application, is easily responsive to or sensitive to heat, and is very well suited to the purpose. In some forms, it has, however, certain objections, *i. e.* it is too sticky or runny, is too easily absorbed by the cork or other filler-body, and is so sticky as to follow the knife of the operator in the act of filling the shoe bottom cavity. It is better, therefore, to introduce with this waxy material or its equivalent, some restraining slow setting component. By the term equivalent I mean to include any binder which is too sticky or active so as to need or be improved by a restrainer or retarder as explained in my parent case, above mentioned. One that I have found very useful for the purpose is an albuminoid, particularly casein, and the combination of a waxy base of a permanently sticky, tenacious, heat-responsive and quick-setting adhesive with an albuminoid, preferably casein, is the subject of my present invention. My filler composition, therefore, broadly stated, as to this feature, consists, in all its essential ingredients, of a body-material and binder mixed to a moldable consistency (when ready for use) and permanently pliable and coherent (when in a thin layer in a shoe-bottom), said binder having a normal free stickiness or adhesiveness which is modified and restrained by an albuminoid. Taking casein

as a type and considering this feature more prominently, a further embodiment of my invention may be defined as a filler consisting of a body-material and a binder united to a moldable consistency, at least at the moment of application in a thin layer in the shoe-bottom, and then coherent, sticky, permanently pliable, and adherent to leather, said binder consisting in whole or in part of a casein solution. Further embodiments or modifications comprise such a filler, in which the casein is less prominent, being united, for example, with a softening oil or medium, or being joined with drying oils, or a filler in which the casein is wholly subordinate to some other ingredient (which may be a softening element) which is relied upon primarily for giving the binder its principal stickiness, etc., such other ingredients being the wax tailings, first mentioned, or the list of substitutes later mentioned herein, or combinations of the same. My filler, in its various aspects, and as made in accordance with these various conditions, is hereinafter explained in detail from these different standpoints. Casein is an albuminoid derived primarily from milk, of which it forms three to four per cent. It is also obtainable to some extent from other sources. Casein is insoluble in pure water but is readily soluble in an alkali or strong acid. It is used preferably in the form of a powder or granules, in the present relation. By one method of use, the casein in the form of powder and in addition to its solvent agents (such, for example, as the wellknown agents borax, soda, sal ammoniac or ammonium carbonate or lime, and the latter's retarding agents fluorid of sodium, etc.) may be mixed with the granulated cork to which may be added the sticky gummy binder or adhesive, usually the resinous residuum of petroleum above mentioned, or wax tailings, though I may use any substitute or combination of the substitutes (or equivalents) mentioned in my former application referred to. The resulting dry granulated mass can thus be shipped to the shoe factories and kept for an indefinite length of time until about to be used. It is then subjected to an addition of cold or warm water or moist steam to develop the latent binding nature of the protein and to render the heat-sensitive wax tailings or other sticky gummy component

more tractable and bring the filler material up to its highest efficiency.

The various solvents capable of bringing about the gelatinizing of the casein may also have a certain fluxing or disintegrating influence upon the gummy sticky component, so that whenever ammoniacal ingredients are used, they will also act as solvents upon the minute parts of the wax-tailings and emulsify the ordinary resins which may form the sticky gummy component of the filler mass. Such solvent assistants for the casein as borax or lime, etc., have no influence upon the wax tailings which is desirable, leaving the latter in proper condition for the mechanical mixing and beating up with the gelatinized casein. Their action upon resins is well known but there are artificial resins offered to the trade which are incapable of saponification but which can be made to form the desired sticky gummy component and can thus be spread in minute parts throughout the mass, as explained. The solvent or dissolving solution for the casein may be added by the shoe manufacturer in the water or liquid vehicle when getting it ready for use, in which case this feature is omitted in the preparation of the approximately dry filler mass. Whenever the solvent is added, as for example a weak solution of soda or ammonium bicarbonate, enough is added to dissolve the casein, and is stirred until the mass becomes uniformly fluid or pasty. Or, the binder may be supplied to the shoe manufacturer in a solution or mixture, requiring the shoe manufacturer simply to add and mix the comminuted cork, or other porous, fibrous or pulpy body material, to the consistency of a stiff, workable dough. Or the binder may be supplied in a semi-plastic condition, like putty, requiring merely treatment with hot water to turn it into a highly effective paste and then admixed with the body material. The casein may be precipitated out by using acids or by formaldehyde, but for my purpose it is better to let it dry in place by gradually losing its water and under the circumstances it appears to have greater efficiency, probably because it is then rather more gelatinous in consistency than when precipitated out. The casein keeps the tailings from penetrating to any great extent the granules of the filler-body material. Unless some restraining agent is used, the tailings may sometimes be absorbed by the body-material to such an extent that the latter will become clogged and heavy and inelastic as when the tailings and cork are mixed first. The viscosity imparted by the casein solution keeps the adhesive from going to the heart of the granules, in practically each of which there remains, therefore, a center of elastic natural fiber which

stays unchanged during the life of the shoe. The fact that the cork is added last may be recognized in the product by the characteristic just explained. Less tailings are therefore needed and the cost correspondingly reduced. This makes it advisable to add the granules after the casein has been gelatinized. I may also omit the alkali water for the casein solution or I may mix the alkali dry in with the tailings and casein, packaging any of these forms to meet the various demands of trade. I may also supplement the casein by additions of one or more of the various substitutes mentioned in my former application, 432,083, viz. starch paste, gluten, gum, dextrin, gelatin, albumin, soluble silicates, or their equivalents. I may replace the tailings in whole or in part by proper substitutes, such as those mentioned in my said former application.

I have explained in my application aforesaid that the sticky component, as for instance wax tailings at a low melting point will sweat through the casein crust after the filler has been installed and while drying out. The resulting combination renders the casein very much less water absorbing and in fact water-repellent. I find that this feature of impregnating the proteid and the semi-solid oily mass with each other is much cheaper and more effective than the setting of the casein by means of acid or formaldehyde.

Casein is capable of making a strong, firm, hornlike binder which can be modified to become less brittle and when mixed with granulated cork can be worked into pliable layers and thus form an excellent filler for shoe cavities. This modifying can be brought about by dissolving the casein in water in addition to the already enumerated solvent assistants, and when the solution of the proteid has been accomplished, I have found that alizarin oil admixed in proper proportions of drying oils (vegetable) will be readily taken up by the casein solution. The resulting binding coating of the granulated cork will be found to be homogeneous and it will also be found that the drying oil has entered into close union with the casein, rendering the latter waterproof without destroying its binding qualities or otherwise impairing its special use. The use of drying oils with a drier in combination with casein is very much different from a use where the casein is acting as the restraining agent of the readily low melting non-drying wax tailings, or where the act is simply one of restraining the too heat-sensitive other binding component.

I have also found the use of casein alone as a binder for granulated cork very serviceable, and when modified by an addition of glycerin, its elasticity as a binder will be

greatly increased. Olein (alizarin) oil may be substituted for the glycerin, and so may other softening oils or fats capable of being fluxed or rendered fluid by means of the soluble oil and when added to a solution of casein will be found to accomplish a like purpose and give to the casein glue a more or less elastic flexible nature. Glycerin gives a toughness and resiliency and olein 10 oil a softness or extra pliability and both of these oily liquids (preferably together) conduce to the waterproofing, etc. Whenever I prepare a shoe filler on the above last described lines and as long as casein 15 or glue or other proteid matter is forming the principal component of the filler-binder, I may use for the application of the material within the shoe bottoms a spreading tool dipped in a solution of formaldehyde 20 or like acting chemical preparation which will influence the proteid matter to render it insoluble in water thereafter on account of acting as a precipitant. Combinations of a large number of ingredients and 25 methods of fluxing and amalgamating the same can be made. I have only enumerated a few and consider the subject broadly covered by my invention.

This invention is subordinate to my Patent No. 945,294, patented January 4, 1910 (application copending with the parent application hereto) and to my other copending application Serial No. 591,207, filed November 7, 1910 since become a Patent No. 35 1,134,931, dated April 6, 1915.

Having described my invention, what I claim as new and desire to secure by Letters Patent is:

1. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution.

2. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution and a softening ingredient.

3. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution and wax tailings.

4. A shoe filler comprising casein, wax tailings, and comminuted filler-body material for a shoe filler.

5. A shoe filler comprising an albuminoid and wax tailings.

6. A shoe filler comprising an albuminoid, wax tailings, and comminuted filler-body material for a shoe filler.

7. The combination, in a shoe-filler, of a permanently sticky, tenacious, slow-drying, waxy adhesive, and a restraining agent consisting at least in part of casein.

8. The combination, in a shoe-filler, of a permanently sticky, tenacious, slow-drying, waxy adhesive, and a restraining agent consisting at least in part of an albuminoid.

9. The combination, in a shoe-filler, of a permanently sticky, tenacious, slow-drying adhesive, casein in solution, and a comminuted filler-body material.

10. A shoe-filler, comprising wax tailings, casein in solution, and comminuted cork, the cork being non-penetrated by the tailings as when added last.

11. A shoe-filler, comprising a permanently sticky tenacious binder, consisting at least in part of wax tailings, and a gelatinized restraining agent containing casein in alkaline solution, and a granular filler-body material.

12. A shoe-filler, comprising a permanently sticky, tenacious binder, containing casein gelatinized by an alkaline solution, and a comminuted filler-body material, the latter being so proportioned and mixed that the absorption of the binder into the particles of the filler-body material is only partial, whereby each of said particles retains a core practically free from the absorbable binder, said core having its natural elasticity practically intact.

13. A shoe filler, consisting of a body-material and a binder united to a moldable consistency, at least at the moment of application in a thin layer in the shoe-bottom, and then coherent, sticky, permanently pliable, and adherent to leather, said binder being responsive to heat at a temperature not injurious to granular cork, and being modified and restrained by an albuminoid, and containing means for maintaining the binder permanently pliable when set in the shoe-bottom.

14. A shoe filler, consisting of a body-material and a binder united to a moldable consistency, at least at the moment of application in a thin layer in the shoe-bottom, and then coherent, sticky, permanently pliable, and adherent to leather, said binder including casein in solution, and means for maintaining the binder pliable when set in a shoe-bottom.

15. A shoe filler, consisting of a body-material and a binder united to a semi-solid, sluggishly moldable consistency, at least at the moment of application in a thin layer in the shoe-bottom, and then sticky, permanently tenacious, pliable, and adherent to

- leather, said binder including casein in solution and containing ingredients for maintaining the binder pliable when set in a shoe-bottom.
- 5 16. A shoe filler, consisting of a body-material and a binder united to a semi-solid, sluggishly moldable consistency, at least at the moment of application in a thin layer in the shoe-bottom, and then sticky, permanently tenacious, pliable, and adherent to leather, said binder including casein in solution and an oily liquid containing at least in part glycerin.
- 10 17. A shoe filler, consisting of a body-material and a binder united to a semi-solid, sluggishly moldable consistency, at least at the moment of application in a thin layer in the shoe-bottom, and then sticky, permanently tenacious, pliable, and adherent to leather, said binder including casein in solution, glycerin and olein oil.
- 15 18. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution and an oily liquid containing olein oil.
- 20 19. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution and an oily, fatty component, all thoroughly mixed together.
- 25 20. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution, and means for rendering the binder water-repellent.
- 30 21. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution, and means for rendering the binder sticky, permanently pliable, and adherent to leather, said binder consisting at least in part of a casein solution, and means for rendering the binder sticky and waterproof.
- 35 22. A shoe-filler, comprising casein in solution, wax tailings, and comminuted filler-body material.
- 40 23. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution, and chemical means for changing the casein solution of the binder into an insoluble protein in the binder when the latter is set.
- 45 24. A shoe filler, comprising a body-material and a binder united to a moldable consistency, at least at the moment of application in a thin layer in the shoe-bottom, and then coherent, sticky, permanently pliable, and adherent to leather, said binder consisting at least in part of a casein solution, chemical means for making the casein solution insoluble in the binder when set, and chemical means for retarding this setting for practical purposes of handling.
- 50 25. A shoe filler, comprising a body-material and a binder united to a moldable consistency, at least at the moment of application in a thin layer in the shoe-bottom, and then coherent, sticky, permanently pliable, and adherent to leather, said binder consisting at least in part of caseinate of lime and a sticky component.
- 55 26. A shoe-filler, comprising casein in solution, a sticky component consisting at least in part of wax tailings, and chemical fluxing means acting to unite into a homogeneous compound both of said ingredients, and comminuted filler-body material.
- 60 In testimony whereof, I have signed my name to this specification, in the presence of two subscribing witnesses.
- ANDREW THOMA.
- Witnesses:
- GEO. H. MAXWELL,  
WALLACE A. SHIPTON.